

## 1

3,118,797

PARTICULATE NITROCELLULOSE COATED WITH  
SORBITAN TRIOLEATE  
Ralph E. Coffee, Alton, Ill., assignor to Glim Mathieson  
Chemical Corporation, a corporation of Virginia  
No Drawing. Filed May 1, 1962, Ser. No. 191,426  
4 Claims. (Cl. 149—10)

This invention relates to improved propellant powder compositions and to improvements in the process for preparing them.

Smokeless powder compositions have been used extensively in the preparation of propellant grains for use in rocket motors, missiles, and gas generating devices of various types. For example, U.S. Patent No. 2,916,775, issued to John J. O'Neill on December 15, 1959, discloses a process for preparing large propellant grains, wherein finely divided particles of nitrocellulose base propellant are mixed with a plastisol solvent consisting of relatively non-volatile nitrocellulose plasticizers to form a flowable paste. The paste is then formed into the shape of a rocket propellant grain and maintained in the shape until consolidated. In processes such as this it is necessary to handle finely divided particles of nitrocellulose powder, which have an average diameter of about 0.003 inch. This powder, because of its small size, is extremely dusty, which causes severe health and safety problems. In order to provide a clean atmosphere in which personnel can work, it is necessary to employ expensive ventilating equipment in the area in which the nitrocellulose powder is handled and processed in a dry form. In addition, the finely divided nitrocellulose particles are very susceptible to the accumulation of static charges which can result in an uncontrolled explosion of the powder. Therefore extreme care must be exercised to avoid the generation of a spark in this material. Furthermore, the finely divided nitrocellulose particles are not readily wetted by the plastisol solvent used in the preparation of the rocket propellant grains. As a result, mixing of the finely divided nitrocellulose particles and plastisol solvent is extremely difficult, since prolonged mixing is necessary to uniformly wet the solid particles with the plastisol solvent and obtain a rocket propellant grain having uniform ballistic properties.

It is the primary object of this invention to overcome the disadvantages inherent in nitrocellulose powder available heretofore.

Another object of the invention is to provide nitrocellulose powder particles which are substantially dust-free while retaining their free flowing characteristics.

Still another object of this invention is to provide an improved astatic propellant powder charge.

Another object of the invention is to provide finely divided nitrocellulose powder particles having improved wettability when contacted with a casting plastisol solvent.

Still another object of the invention is to provide a method of inhibiting foam formation in globular propellant powder processes while producing a solidified powder that is substantially dust-free.

It has now been discovered that when nitrocellulose powder in finely divided form is coated with sorbitan trioleate to yield a substantially complete uniform coating or layer of sorbitan trioleate on each particle of the nitrocellulose powder, the nitrocellulose powder maintains its free flowing properties, but dusting and accumulation of static charges on the nitrocellulose powder are substantially minimized.

The proportion of sorbitan trioleate on the surface of the particles of nitrocellulose powder is maintained between about 0.02 percent and about 0.5 percent by weight of the nitrocellulose powder. When the proportion of

## 2

sorbitan trioleate is less than about 0.02 percent by weight of the powder, generally there is insufficient sorbitan trioleate present to impart the desired improvements in the dusting and static properties of the nitrocellulose powder.

On the other hand when the proportion of sorbitan trioleate on the powder surfaces is greater than about 0.5 percent by weight, little additional improvement is obtained in the dusting and static properties, and the excess sorbitan trioleate acts as a diluent for the nitrocellulose powder.

When sorbitan trioleate is admixed with nitrocellulose powder particles in the above-mentioned range, a sufficient amount of sorbitan trioleate is present to impart a substantially complete uniform coating or layer of sorbitan trioleate on each particle of nitrocellulose powder. The sorbitan trioleate has no appreciable solvent effect upon the nitrocellulose, and it does not penetrate the exterior surfaces of the grain, but instead is present only as an external coating having approximately a molecular thickness.

Sorbitan trioleate may be applied to the surfaces of the nitrocellulose powder in any convenient manner that will yield a substantially complete uniform coating or layer of the sorbitan trioleate on the exterior surfaces of the nitrocellulose powder particles. Thus, the nitrocellulose

particles can be mixed with the sorbitan trioleate in the above defined proportions in a suitable tumbling apparatus, with or without water. If desired, the nitrocellulose powder particles and/or the sorbitan trioleate can be mixed with water prior to the coating operation. In one embodiment of the invention, an aqueous slurry or suspension of nitrocellulose powder particles to be coated is admixed with an aqueous emulsion or suspension of sorbitan trioleate in a continuous process. This is most readily accomplished by dewatering an aqueous slurry of

the nitrocellulose powder particles in a continuous centrifuge, and then adding an aqueous emulsion of sorbitan trioleate to the centrifuge. The emulsified sorbitan trioleate readily replaces the water wetting the nitrocellulose powder, and the excess emulsion is conveniently removed

from the powder charge by continued centrifugation. Any water remaining on the powder grains can then be removed by conventional drying methods.

The novel coating technique of the instant invention is particularly suitable for use in conventional ball powder processes wherein a lacquer of nitrocellulose dissolved in a suitable solvent, is dispersed in an aqueous medium to form globules of the nitrocellulose lacquer, and the solvent is then evaporated from the globules to form solidified particles of nitrocellulose.

Prior to the hardening process, protective colloids such as animal bone glue are added to the lacquer suspension, which may cause considerable frothing or foaming of the suspension. Such frothing adversely affects the operation of the pumps, agitators, and other equipment employed in the process. However frothing is substantially eliminated, and the desired coating is effected when sorbitan trioleate is added in the above defined proportions to the

hardening step in conventional nitrocellulose powder processes. For example, when sorbitan trioleate is added to the flash chamber in the process described in U.S. Patent No. 2,888,713, issued June 2, 1959, to Ralph L. Cook and Eugene A. Andrew, or to the still in U.S. Patent No. 3,014,246, issued December 26, 1961, to the same inventors, frothing is substantially eliminated, and the solidified nitrocellulose particles produced in these processes, when combined with the sorbitan trioleate addition of the instant invention, has a substantially complete uniform layer of sorbitan trioleate on the exterior surfaces.

The size or shape of the nitrocellulose powder particles is immaterial, but the instant novel invention is utilized more advantageously with spherical nitrocellulose powder

grains having an average diameter of between about 0.0002 and about 0.004 inch. Nitrocellulose particles of this size are used as the base material in the manufacture of giant rocket grains and the like. Although the present invention is concerned primarily with the treatment of such casting powder, the qualities of standard small arms ammunition propellant are also materially improved when coated with sorbitan trioleate in accordance with the instant invention. Sorbitan trioleate can be used to replace or augment conventional graphite glaze on commercial and military nitrocellulose powders.

When nitrocellulose powder particles coated with sorbitan trioleate in accordance with this invention are used as a base material in the manufacture of rocket grains, the nitrocellulose particles are mixed with a plastisol solvent which has relatively poor solvent power for the nitrocellulose at ordinary room temperature, but which is very rapid acting and has a relatively great solvent power at elevated temperatures, for example at temperatures above about 60° C. The plastisol solvent can be either a deterrent or an energizing modifier, or a mixture of energizing modifier and deterrent. Suitable energizing modifiers include nitroglycerine, triethylene glycol dinitrate, butane triol trinitrate, diglycol dinitrate, ethylene glycol dinitrate, and the like. Suitable deterrents that may be employed include dibutyl phthalate, dimethyl sebacate, dibutyl succinate, dibutyl adipate, dipropyl adipate, triacetine, ethyl diphenyl phosphate, tributyl phosphate and the like. Sorbitan trioleate of the instant invention is readily compatible with plastisol solvents of this type and its use markedly reduces the time required for obtaining a uniform plastisol mixture. In addition, sorbitan trioleate has no appreciable solvent power for nitrocellulose powder, and does not adversely affect the "pot life" of the plastisol mixture.

In order that the invention may be further illustrated, the following examples are presented without any intention of being limited thereby. All parts and percentages are by weight unless otherwise specified.

#### Example I

Nitrocellulose lacquer was prepared by adding about 1.5 parts of nitrocellulose-water mixture (1 part nitrocellulose and 0.5 part water) to 4 parts of ethyl acetate containing about 1 percent 2-nitrodiphenylamine and about 0.25 percent of chalk. These materials were then mixed at a temperature of about 65° C. for about 1/2 hour to form a substantially homogeneous lacquer. In a separate vessel a suspending medium was prepared by admixing 3.4 percent sodium sulfate, 1.7 percent animal glue, 0.5 percent ethyl acetate, 0.00235 percent sorbitan trioleate with water. The resulting mixture was then heated to about 65° C. with agitation until substantially complete dissolution was effected.

The nitrocellulose lacquer and the aqueous suspending medium were separately fed to a grainer of a type similar to that shown in FIGURE 2 of U.S. Patent No. 3,014,246. The nitrocellulose lacquer was fed to the grainer at a rate of about 1/2 that of the aqueous suspending medium. The nitrocellulose lacquer was divided by the rotating blades of the grainer into fine globules having an average diameter of about 0.010 inch, and the resulting granules were uniformly suspended throughout the aqueous suspending medium. A portion of the resulting aqueous suspension of globules was continuously withdrawn from the grainer and admixed with additional aqueous suspending medium (in a ratio of 5 parts to 1 part of the original suspension) which had been heated to a temperature of about 128° C. and was under a pressure of about 40 p.s.i. The diluted aqueous globule suspension was then passed through an orifice into a flash chamber maintained as slightly below atmospheric temperature. Ethyl acetate and some water vapor were evaporated from the diluted aqueous globule suspension

when the pressure of the aqueous suspension was reduced. Substantially no foaming occurred in the flash chamber due to the presence of sorbitan trioleate. These vapors were removed from the flash chamber under a slight vacuum. Due to evaporation of the ethyl acetate, the globules in the aqueous medium were solidified into gelatinized nitrocellulose particles. The resulting slurry of these particles, which were coated with a thin substantially continuous layer of sorbitan trioleate, was fed to a centrifuge to remove the aqueous medium. The particles were then washed with water and heated to dryness. The dried nitrocellulose particles contained about 0.2 percent sorbitan trioleate as a coating. The coated particles had a diameter between about 0.0002 and 0.004 inch, but were not dusty when stirred in the atmosphere.

#### Example II

The superior defoaming properties of sorbitan trioleate were demonstrated in a series of comparative tests using an aqueous solution containing about 3.4 percent sodium sulfate, about 1.7 percent animal glue, and about 0.5 percent ethyl acetate.

One drop of sorbitan trioleate was added to 25 milliliters of the aqueous solution in a 50 milliliter test tube and the test tube was stoppered and vigorously shook eight times. The resulting foam completely dissipated in less than 5 seconds.

For purposes of comparison, when the procedure was repeated, using one drop of sorbitan monooleate instead of sorbitan trioleate, more than 60 seconds were required before the foam completely dissipated.

For purposes of further comparison, the procedure was repeated with the exception that nothing was added to the standard solution prior to shaking. Fifty-two seconds were required for the foam to completely dissipate in this instance.

While the invention has been described in detail with respect to the coating of nitrocellulose particles it will be recognized by those skilled in the art that nitrocellulose may be used alone or in combination with deterrents such as dinitrotoluene, dialkyl and diaryl phthalates, and the like. In addition energizers such as nitroglycerine, aluminum, trinitrotoluene, cyclotrimethylenetrinitramine, ammonium perchlorate, and the like can also be incorporated with the nitrocellulose or mixed with the surface coated powder. Whenever desirable, the nitrocellulose can be replaced in whole or in part by other gelatinizable polynitro materials such as nitro starch, polyvinyl nitrate, and other similar materials.

It will be recognized by those skilled in the art that various modifications, some of which have been referred to above, may be made in the invention without departing from the spirit thereof.

Having thusly described the invention, what is claimed and desired to be secured by Letters Patent is:

1. Nitrocellulose particles coated with sorbitan trioleate in a proportion equivalent to between about 0.02 and about 0.5 percent by weight of the nitrocellulose, the coating of sorbitan trioleate being substantially complete and of substantially uniform thickness.

2. The process for preparing substantially dustless nitrocellulose particles which comprises admixing nitrocellulose particles with sorbitan trioleate in a proportion equivalent to between about 0.02 percent and about 0.5 percent by weight of the nitrocellulose, and continuing the mixing until a substantially complete layer of sorbitan trioleate is formed on the outer surfaces of the nitrocellulose particles.

3. The process of claim 2 wherein sorbitan trioleate is mixed with the nitrocellulose particles as an aqueous dispersion.

4. In the process for preparing solidified nitrocellulose particles wherein lacquer globules of nitrocellulose in a solvent are suspended in an aqueous non-solvent medium to yield a suspension of the globules, the suspension is

subjected to a temperature above the boiling point of the solvent and a pressure sufficient to prevent boiling of the solvent at the temperature employed, the resulting suspension is conveyed to a reduced pressure zone where temperature and pressure conditions are such that the solvent is evaporated from the globules to yield an aqueous suspension of solidified particles of gelatinized nitro-cellulose, and the solidified particles are then separated from the aqueous suspension, the improvement which comprises adding sorbitan trioleate to the suspension of lacquer globules in a proportion equivalent to between 10

about 0.02 and about 0.5 percent by weight of nitrocellulose contained therein, whereby foaming is inhibited in the reduced pressure zone and said solidified particles are substantially dustless.

References Cited in the file of this patent

UNITED STATES PATENTS

2,771,351 Holmes ----- Nov. 20, 1956

FOREIGN PATENTS

579,302 Great Britain ----- July 30, 1946

UNITED STATES PATENT OFFICE  
CERTIFICATE OF CORRECTION

Patent No. 3,118,797

January 21, 1964

Ralph E. Coffee

It is hereby certified that error appears in the above numbered patent requiring correction and that the said Letters Patent should read as corrected below.

Column 3, line 73, for "as" read -- at --; column 4, line 3, for "triolate" read -- trioleate --; lines 62 and 63, for "introcellulose" read -- nitrocellulose --.

Signed and sealed this 23rd day of June 1964.

(SEAL)  
Attest:

ERNEST W. SWIDER  
Attesting Officer

EDWARD J. BRENNER  
Commissioner of Patents